

## UNITED STATES PATENT OFFICE.

LEWIS EDGAR ODELL, OF NEW ROCHELLE, NEW YORK, ASSIGNOR TO W. A. MOORE, OF NEW YORK, N. Y.

## LIQUID COATING COMPOSITION.

No. 893,010.

Specification of Letters Patent.

Patented July 14, 1908.

Application filed February 7, 1907. Serial No. 356,195.

To all whom it may concern:

Be it known that I, LEWIS EDGAR ODELL, residing at New Rochelle, in the county of Westchester and State of New York, have 5 invented certain new and useful Improvements in Liquid Coating Composition, of which the following is a full, clear, and exact description, such as will enable others skilled in the art to which it appertains to make and 10 use the same.

This invention relates broadly to a process and means for coating various building materials, but since certain advantages characteristic of the invention prominently appear when it is resorted to for the purpose of preserving wood it will be conducive to clearness to describe an embodiment thereof as applied in such connection.

One object of this invention is to formulate 20 a commercially practicable method of preserving wood which is adapted for being very readily carried out at a low cost.

Another object contemplated by this invention is to obtain a certain new and improved 25 preservative whose ingredients will be cheap and readily obtainable, and which when applied will very effectively accomplish its purpose.

Other objects and advantages will be in 30 part obvious and in part pointed out hereinafter.

This invention accordingly consists in the several steps and the relation and order of one or more of such steps with relation to 35 each of the others thereof which will be exemplified in the process hereinafter described, and the scope of the application of which will be indicated in the following claims.

More specifically, this invention proposes a 40 coating composition comprising an alkaline agent such as slaked lime, and a preservative such as charcoal. These ingredients will preferably be suspended in a suitable liquid carrier which is well adapted to penetrate the 45 pores of wood so as to impregnate the same with the composition.

In preparing the coating composition the lime may be slaked and mixed with boiled linseed oil or turpentine, and to this emulsion 50 will be added finely powdered carbon, which may be in the form of charcoal, lamp black or any of the other commercially ob-

tainable equivalents. These ingredients will be intimately ground together and thoroughly emulsified with the carrier so as to 55 form a smooth flowing paint.

It is to be understood that various proportions of the foregoing ingredients may be employed—thus 46 parts of lime may be mixed with 54 parts of charcoal, and sufficient oil will be employed to form a freely 60 flowing paint, and it is also to be understood that in some cases other materials may also be added, but the foregoing embodiment is that which will ordinarily be preferable to 65 employ in practice, and is regarded as representing substantial improvements over the many implied and obvious variations of the same.

In applying this paint, which in practice 70 will be found to be of a grayish color, the wood will preferably be in a relatively dry state, and the paint may be applied directly thereto so as to thoroughly impregnate and cover the superficial surface of the wood. 75 This impregnation may be accomplished in several ways, and in some cases may be forced into the pores of the wood through the application of external pressure. It is also proposed to successively apply a series of 80 coatings of paint prepared in the foregoing manner. Thus, the first coating may be comparatively thin, so that a very perfect impregnation may be secured, and the subsequent coatings may be successively thicker 85 so as to give body to the surface.

It will thus be seen that this invention is characterized by the greatest of simplicity, and that the various ingredients thereof are exceedingly cheap. In practice it will be 90 found that wood coated in accordance with this invention will be very effectively preserved against decay throughout long lapses of time, and that but little skill will be required for preserving wood in accordance 95 with the invention.

Having described my invention, what I claim as new and desire to secure by Letters Patent is:—

1. A preservative coating composition 100 which constitutes an emulsion consisting of oil, powdered charcoal, and a pulverulent alkaline material.

2. A preservative coating composition

505.4

X327

X3215

which comprises slaked lime, a neutral pul-  
verulent carbonized material, and an oily car-  
rier holding said ingredients in suspension.

3. A preservative coating composition  
5 which comprises approximately 46 parts of  
powdered lime to 54 parts of powdered char-  
coal, and an oily carrier.

4. A preservative coating composition  
which comprises approximately of 46 parts of

powdered lime, approximately 54 parts of a 10  
powdered carbonized material, and a liquid  
carrier.

In testimony whereof I affix my signature,  
in the presence of two witnesses.

LEWIS EDGAR ODELL.

Witnesses:

ALFRED SCHACHAT,  
CHARLES J. DUNLAP.